

## UNITED STATES PATENT OFFICE

2,075,742

SHAPED BODIES MANUFACTURED FROM  
AN ALLOY OF TUNGSTEN CARBIDE OR  
MOLYBDENUM CARBIDEKurt Moers, Berlin-Steglitz, Germany, assignor  
to General Electric Company, a corporation  
of New YorkNo Drawing. Application May 22, 1935, Serial  
No. 22,784. In Germany June 1, 1934

7 Claims. (Cl. 75—136)

This invention relates to shaped bodies manufactured from an alloy of tungsten carbide or molybdenum carbide and an auxiliary metal of the iron group having a lower fusion point.

5 In order to impart an increased density to sintered hard metal alloys composed of tungsten carbide or molybdenum carbide and an auxiliary metal of lower fusion point, it has already been proposed to subject at glowing temperature 10 to a mechanical treatment, such as hammering, rolling, pressing and so on, the shaped bodies made from the powdered alloy components by pressing. This proposal, however, has not been

realized hitherto in practice because of the fact 15 that the red-hot shaped bodies due to their coming into contact with air during the mechanical treatment not only burn and scale, but also lose part of their carbon content and show a decrease of their surface hardness. In addition, as such 20 shaped bodies mainly consist of the very hard tungsten carbide or molybdenum carbide, they are not sufficiently plastic even when heated, and therefore cannot be mechanically treated without the risk of formation of cracks.

25 In order to overcome these drawbacks, according to the present invention an alloy is made use of for the manufacture of shaped bodies to be produced by pressing, sintering and a subsequent mechanical treatment, which alloy, true is 30 likewise composed of tungsten carbide or molybdenum carbide and a metal of the iron group of lower fusion point, but, further, has an addition of 1-5% of titanium carbide, while the percentage of the auxiliary metal of the iron group 35 amounts to 25-40%.

In general, with sintered hard metal alloys built up on the basis of tungsten carbide or molybdenum carbide only an addition of auxiliary metal of up to 20% is made, because a higher percentage of auxiliary metal, which in itself has 40 likewise been suggested, would cause an undesired decrease of the properties of strength of the alloy. In the alloy used according to the invention for the manufacture of the new shaped bodies the 45 higher content of auxiliary metal of 25-40% serves merely to render the alloy more ductile during the mechanical treatment. The lower strength which, it is true, is caused by this high percentage of auxiliary metal, is wholly compensated by the addition of titanium carbide which has a hardening effect. This addition has the further effect that any oxidation, scaling or burning of the carbon of the alloy, which occurs 50 by the contact of the redhot shaped bodies with the air, is completely eliminated. Spite of their

comparatively high percentages of auxiliary metal, alloys composed in accordance with the invention and containing for example 68% WC, 30% Fe and 2% TiC or 33% WC, 33% MoC, 30% Co and 4% TiC show Rockwell hardness of 85-86, that is, Rockwell hardness which comes very near to those of the hardest sintered carbide alloys. The density of shaped bodies made from the present alloys, however, is notably higher, so that these shaped bodies in use wear away to a much less extent.

After the problem has been solved by the present invention, viz. to shape hard metal alloys plastically without any substantial detraction of the hardness, it is now possible to give the hard 15 metal alloys the shape of plates, strips or wires which owing to the preceding mechanical treatment are able to withstand elastic stresses. Thus, according to the invention hard metal alloys can be shaped to knives and razor blades or to 20 grinding mortars, fittings and the like. Flat and plate-shaped bodies manufactured from alloys according to the invention are well suited for many purposes, for example as inserts for the walls of safes strong boxes and the like.

25 I claim:

1. Shaped bodies produced by pressing, sintering and a subsequent mechanical treatment from an alloy containing 25% to 40% of an auxiliary metal of the iron group, 1% to 5% of titanium carbide, the remainder consisting of tungsten carbide.

2. Shaped bodies produced by pressing, sintering and a subsequent mechanical treatment from an alloy containing 25% to 40% of an auxiliary metal of the iron group, 1% to 5% of titanium carbide, the remainder consisting of molybdenum carbide.

3. Shaped bodies produced by pressing, sintering and a subsequent mechanical treatment from an alloy containing 25% to 40% of an auxiliary metal of the iron group, 1% to 5% of titanium carbide, the remainder of the alloy consisting of tungsten carbide and molybdenum carbide.

4. Shaped bodies produced by pressing, sintering and a subsequent mechanical treatment from an alloy containing 25-40% of an auxiliary metal of the iron group, 1-5% of titanium carbide, the remainder consisting of material from the group tungsten carbide and molybdenum carbide.

5. Shaped bodies produced by pressing, sintering and a subsequent mechanical treatment, said bodies comprising an alloy consisting substan-

5

15

20

25

30

35

40

45

50

55

tially of 68% tungsten carbide, 30% iron, 2% titanium carbide.

6. Shaped bodies produced by pressing, sintering and a subsequent mechanical treatment, said bodies comprising an alloy consisting substantially of 33% tungsten carbide, 33% molybdenum carbide, 30% cobalt and 4% titanium carbide.

7. A sintered alloy containing about 25% to 40% of metal of the iron group, about 1% to 5% titanium carbide, the remainder of said alloy consisting substantially of carbide material from the group tungsten carbide and molybdenum carbide.

KURT MOERS.